

United States Patent [19]  
Franks et al.

[11] 3,917,518  
[45] \*Nov. 4, 1975

[54] HYPOCHLORITE PRODUCTION

[75] Inventors: **Charles R. Franks**, North Madison;  
**Barry A. Schenker**, Mayfield  
Heights; **James M. Kolb**, Mentor, all  
of Ohio

[73] Assignee: **Diamond Shamrock Corporation**,  
Cleveland, Ohio

[\*] Notice: The portion of the term of this  
patent subsequent to Feb. 19, 1991,  
has been disclaimed.

[22] Filed: **Apr. 19, 1973**

[21] Appl. No.: **352,419**

[52] U.S. Cl. .... **204/95**; 204/290 F

[51] Int. Cl.<sup>2</sup> .... **C25B 1/24**

[58] Field of Search .... **204/95, 290 F**

[56] References Cited

UNITED STATES PATENTS

1,397,239 11/1921 Slater ..... 204/95

|           |         |                       |           |
|-----------|---------|-----------------------|-----------|
| 3,627,669 | 12/1971 | Entwistle et al. .... | 204/290 F |
| 3,684,543 | 8/1972  | DeNora et al. ....    | 204/290 F |
| 3,711,397 | 1/1973  | Martinsons ....       | 204/290 F |
| 3,732,157 | 5/1973  | DeWitt ....           | 204/95    |
| 3,776,834 | 12/1973 | O'Leary ....          | 204/96    |
| 3,779,889 | 12/1973 | Loftfield ....        | 204/95    |
| 3,793,164 | 2/1974  | Kolb et al. ....      | 204/99    |

Primary Examiner—Oscar R. Vertiz

Assistant Examiner—Wayne A. Langel

Attorney, Agent, or Firm—Timothy E. Tinkler

[57] ABSTRACT

A process is described that is particularly applicable to the continuous production of hypochlorite solution over long periods of time by electrolysis of aqueous chloride solutions with an anode having a coating that is a mixture of oxides of tin, antimony, at least one platinum group metal, and a valve metal selected from the group titanium and tantalum, all in certain proportions.

4 Claims, No Drawings

## HYPOCHLORITE PRODUCTION

## BACKGROUND OF THE INVENTION

A variety of uses for alkali metal hypochlorite solutions, including bleaching and disinfecting, are known. One widespread use is for microbiocidal applications in sewage and water treatment facilities, where there is considerable demand for units capable of on-site generation of hypochlorite solutions, thereby eliminating the need for expensive shipping of dilute solutions or the sometimes hazardous handling and storage of chlorine gas. Such units must, of course, be relatively maintenance free to allow their convenient use.

To this end, compact and efficient cell units in a variety of sizes have been designed. A primary problem with such units, however, has been to achieve operation, either continuously or intermittently, over long periods of time without need for maintenance or replacement of cell components. A particular problem has been to obtain a cell and process for operating same wherein the useful lifetime of the anodes of said cell is sufficient to allow relatively maintenance free operation.

## STATEMENT OF THE INVENTION

Therefore, it is an object of the present invention to provide an efficient process for the production of hypochlorite solutions by electrolysis.

It is a further object of the present invention to provide an efficient process for the electrolytic production of hypochlorite, which process allows long-term operation without anode replacement.

These and further objects of the present invention will become apparent to those skilled in the art from the specification and claims that follow.

There has now been found in a process for the production of hypochlorite by the electrolysis of an aqueous alkali metal chloride solution, the improvement that comprises passing an electrolyzing current through said solution between a cathode and an opposed anode, which anode comprises a conductive base bearing on at least a portion of the surface thereof a mixed oxide coating of from 30 to 90 percent stannic oxide, 1.0 to 10 percent antimony oxide, 1.0 to 50 percent of at least one platinum group metal oxide, and 0.5 to 30 percent of a valve metal oxide selected from the group consisting of titanium and tantalum oxides, with the proviso that the mole ratio of tin to antimony oxides is between 95:5 and 85:15. Such a process is characterized by efficient hypochlorite generation over long periods of useful anode life. Anode life is determined by the length of time required for the anode to "passivate". An anode is considered passivated when the voltage at which the desired electrolytic reaction occurs becomes so high as to prohibit further practical operation, e.g., in excess of 8 volts in a hypochlorite cell.

## DESCRIPTION OF THE PREFERRED EMBODIMENTS

Basically, the invention is concerned with a process for the production of an alkali metal hypochlorite solution by the electrolysis of an alkali metal chloride in a diaphragmless cell. The cell configuration is not critical to the practice of the present invention except in that it must be adapted for operation with dimensionally stable electrodes. Thus, any known cell may be used, such cells comprising an enclosure provided with an

electrolyte inlet and an outlet for electrolyte and product and containing at least one anode and one cathode opposed to each other in a substantially parallel relationship. The cell may be of either the monopolar design, that is, wherein there is a separate external electrical connection for each electrode, or bipolar in configuration, wherein the current passes, from a terminal anode through a plurality of bipolar electrodes disposed between said terminal anode and a terminal cathode at the opposite end of the cell. Within the cell, in the absence of a diaphragm, the products of electrolysis, i.e., chlorine and alkali metal hydroxide, immediately mix to form the desired hypochlorite solution.

A critical feature of the invention is the use of a particular anode which, as mentioned above, is a conductive substrate bearing on at least a portion of the surface thereof a coating of mixed oxides of tin, antimony, at least one platinum group metal, and a valve metal selected from the group titanium and tantalum. With the use of such anodes, the tendency towards passivation when oxygen is evolved at the anodic surface is greatly reduced and hence the anodes exhibit a long useful lifetime.

The conductive substrate is preferably titanium, although tantalum, niobium, and zirconium may also be employed. In addition, a covering of one of the aforementioned metals over a more conductive material, such as copper or aluminum, may be employed. Further, layers on the substrate intermediate the base metal and the coating, such as those described in U.S. Pat. No. 3,711,397, are contemplated. The configuration of the substrate may vary considerably but is generally in the form of an imperforate or foraminous sheet, e.g., expanded titanium metal.

What may be considered the first of the components in the coating composition is stannic oxide, preferably present in the form of crystalline  $\text{SnO}_2$  and employed within the range of from 30 to 90 percent by weight of the total coating composition.

The antimony oxide component enters into the tin oxide crystal lattice, rendering same more electrically conductive. Although the antimony is present in an indeterminate oxide form owing to its entrance into the stannic oxide crystal lattice, it is expressed for convenience sake as  $\text{Sb}_2\text{O}_3$ . Thus, on this basis, the antimony oxide is present within the range from 1.0 to 10, preferably 4.0 to 10, percent by weight.

The foregoing ranges of tin and antimony oxides are further qualified by the proviso that they be present, respectively, in the range, on a mole ratio basis, of 95:5 to 85:15, especially 90:10. In this fashion, there is obtained the desired doping effect of the antimony on the tin oxide without the presence of an excess separate phase of antimony oxide.

The third component of the mixed coating is "at least one platinum group metal oxide", by which term it is intended to include the oxides of platinum, palladium, ruthenium, iridium, rhodium, and osmium, especially those of ruthenium and iridium. These platinum group metal oxides are present for the most part in their most highly oxidized state and within the range of from 1.0 to 50 percent by weight. An especially preferred anode is one the coating of which contains a combination of  $\text{RuO}_2$   $\text{IrO}_2$  or rhodium oxide.

The final component is a valve metal oxide selected from the group consisting of titanium and tantalum oxides. Whereas the titanium is present in the form of

$TiO_2$  and is essentially crystalline (rutile) in nature, when tantalum is employed, a generally amorphous tantalum oxide results. Therefore, although it is expressed as  $Ta_2O_5$ , it is understood that mixtures of tantalum oxides may in fact be present. The amounts of a valve metal oxide employed are generally within the range of from 0.5 to 30 percent by weight.

While many of the variety of methods known for producing mixed metal oxide coatings may be employed, the preferred method of preparing the multicomponent coating composition on the titanium substrate is by deposition from a solution of the appropriate thermally decomposable salts. For example, it is desirable to paint or brush an acidified alcoholic solution of said salts onto the substrate followed by drying at 100°–140° C for from 3 to 10, especially 5, minutes and finally by baking in an oxidizing atmosphere, e.g., air, at 450° to 520° C, especially 500° C, for from 5 to 10, especially about 7, minutes. This procedure may then be repeated any number of times until the desired coating thickness is obtained, for example, 6 to 10 coats. The preferred solvents for the thermally decomposable salts are the lower alkanols such as ethanol, propanol, amyl alcohol, and especially n-butyl alcohol, although other solvents including water may be employed. To these solvents there is generally added from 0 to 50 percent by volume of an acid, such as hydrochloric acid. The concentration of the metals in the solution from which the coating composition is to be formed ranges between about 50 and 200 grams per liter. The salts employed are generally any thermally decomposable inorganic or organic salt or organic ester of the metals in question, such as the chlorides, nitrates, alkoxides, alkoxy halides, resinate, amines, and the like. Specific and illustrative examples include potassium hexachloroplatinate, hexachloroiridic acid, ruthenium trichloride or tribromide, orthobutyl titanate, antimony trichloride or pentachloride, and stannic chloride or dibutyl tin dichloride.

It will be understood by those skilled in the art that it is possible to use a number of combinations of preformed oxides of the various component metals and salts of the remaining materials, although it is generally believed that preformed valve metal oxides should not be employed nor should separately preformed tin and antimony oxides be used. Further, if thermal decomposition is incomplete, small amounts of salts may remain without detrimental effect in the coating, for example, small amounts of chloride in the primarily oxide coating.

The cathode, again, is not critical to the practice of the present invention, any of those conventionally employed being satisfactory. A preferred material is titanium, although steel, stainless steel, or titanium bearing an electrocatalytically active, electrically conductive coating, such as a mixed titanium dioxide-ruthenium dioxide coating, may be employed. Configuration is not critical to the process but rather is a consideration of the cell design. Generally a continuous sheet is employed. Of course, in the instance of a bipolar electrode, the substrate for the anode (e.g., titanium) may also serve on its opposite face as the cathodic surface or a laminate of the appropriate metals may be employed.

While the interelectrode gap may be within the range of 0.04–0.125 inch, the lower gaps are generally preferred for efficient operation.

The solution to be electrolyzed is an aqueous alkali metal chloride, especially a solution containing from about 28–35 grams per liter of alkali metal chloride. When the solution is made by dissolving relatively pure alkali metal chlorides in water, the use of solutions having a, for example, sodium chloride content in excess of 35 gpl, is uneconomic. On the other hand, concentrations substantially less than about 28 gpl sodium chloride provide solutions in which excessive amounts of oxygen are generated at the anode, thereby accelerating passivation. Rather than electrolyze an artificial alkali metal chloride solution, it is quite possible and indeed economically desirable to employ sea water as the electrolyte since the appropriate salt concentration is already present. It will be understood that, owing to the presence of various contaminants, e.g., calcium and magnesium ions, special precautions, such as periodic flushing of the cell, will be necessary to prevent buildup of undesired deposits. Obviously, for economic reasons, the term "alkali metal" in this context refers mainly to potassium and especially sodium.

The temperature at which electrolysis is conducted should be within the range of from 5° to 50° C, especially 15°–30° C. At temperatures in excess of this range, the chemical conversion of hypochlorite to chlorate is favored, thus reducing efficiency. On the other hand, at low temperatures, the relative overvoltages of oxygen and chlorine are displaced with the result that larger quantities of oxygen are evolved, again attributing to more rapid anode passivation.

The pH at which the hypochlorite-forming reaction proceeds is within the range of from about 7 to 10. At a lower pH, the chlorate-forming reaction is preferred while higher ranges must be artificially induced and serve no economic purpose. Generally, it will be found that there is no need to adjust the electrolyte to obtain the desired pH since a salt solution of the appropriate concentration will on establishment of electrolysis equilibrate at a pH within the range of 9.0–9.5.

Generally, concentrations of alkali-metal hypochlorite within the range of about 0.5 to 10 grams per liter are contemplated. In the instance where salt must be purchased and dissolved to provide the electrolyte, it is desirable to control the flow rate and other reaction conditions so that a concentration of hypochlorite within the range of from 8 to 10 grams per liter is achieved, thus avoiding a waste of the relatively expensive alkali metal chloride. On the other hand, where sea water is the electrolyte, cost of the alkali metal chloride is not a consideration and concentrations within the range of 0.5 to 2.0 gpl are economical. To this end, while recirculation may be employed, it is more feasible to dictate the hypochlorite concentration by controlling the flow rate through the cell. Since the amount of available chlorine required by the average sewage treatment plant is only on the order of 10 ppm and only a 2 ppm concentration is required in the waters of cooling towers, it will be apparent that any of the concentrations obtained by the invention are useful.

Typically, the process is operated at a relatively low current density, e.g., within the range of from about 0.5 to 1.0 ampere per square inch. While at higher current densities, the production rate is increased somewhat, this is offset by the decrease in useful anode life. On the other hand, a low current density generally results in a low current efficiency. Hence, an increase in electrode area must be provided to achieve a like production.

Thus, a balance is struck within the above-stated range.

In summary, a preferred process for the production of solutions having a sodium hypochlorite concentration within the range of **0.5** to **10** gpl comprises passing an electrolyzing current of between **0.5** and **1.0** asi through an aqueous solution having a pH of greater than 7 and containing **28** to **35** gpl sodium chloride at a temperature from **5°** to **50°** C between a cathode and an opposed anode, which anode comprises a titanium substrate bearing on at least a portion of the surface thereof a coating of the mixed oxides of tin, antimony, at least one platinum group metal, and a valve metal selected from the group consisting of titanium and tantalum.

In order that those skilled in the art may more readily understand the present invention and certain preferred embodiments by which it may be carried into effect, the following specific examples are afforded.

#### EXAMPLE 1

An anode coating solution is prepared by dissolving **25** grams  $\text{SnCl}_4 \cdot 5\text{H}_2\text{O}$ , **1.8** grams  $\text{SbCl}_3$ , **5.3** grams  $\text{RuCl}_3 \cdot x\text{H}_2\text{O}$  (38% Ru), and **0.86** gram orthobutyl titanate in **25** ml butanol and **12.5** ml HCl (36%). A titanium sheet is coated by brushing with this solution followed by drying at **110°** C for **3** minutes and baking in air at **500°** C for **7** minutes. The procedure is repeated until a coating containing **0.64** gram per square foot of ruthenium is attained. The resultant electrode has the following composition, calculated on the indicated oxide weight basis: **73.1%**  $\text{SnO}_2$  **7.8%**  $\text{Sb}_2\text{O}_3$ , **17.5%**  $\text{RuO}_2$ , and **1.6%**  $\text{TiO}_2$ .

The electrode is disposed as the anode in an electrolytic cell opposite and spaced **0.04** inch apart from a titanium metal cathode. Electrolysis of a **28** to **30** gram per liter aqueous sodium chloride solution having a temperature of **5°** C is conducted for **235** hours at an anode current density of **1** asi before the voltage increases to in excess of **8**, indicating passivation.

#### EXAMPLE 2

Example 1 is repeated, the anode coating in this in-

stance being **47.2%**  $\text{SnO}_2$ , **5.3%**  $\text{Sb}_2\text{O}_3$ , **27.3%**  $\text{RuO}_2$ , and **20.2%**  $\text{Ta}_2\text{O}_5$ , and an anode lifetime of **153** hours is obtained.

We claim:

**1.** In a process for the production of hypochlorite by the electrolysis of an aqueous alkali metal chloride solution, the improvement that comprises passing an electrolyzing current through said solution between a cathode and an opposed anode, which anode comprises a conductive base bearing on at least a portion of the surface thereof a coating consisting essentially of from **30** to **90** percent by weight stannic oxide, from **1.0** to **10** percent antimony oxide, calculated as  $\text{Sb}_2\text{O}_3$ , from **1.0** to **50** percent of at least one platinum group metal oxide and from **0.5** to **30** percent of a valve metal oxide selected from the group consisting of titanium and tantalum oxides, with the proviso that the mole ratio of  $\text{SnO}_2:\text{Sb}_2\text{O}_3$  is between **95:5** and **85:15**.

**2.** A process for the production of a solution containing from **0.5** to **10** grams per liter of hypochlorite, which process comprises passing an electrolyzing current through an aqueous solution of alkali metal chloride, at a pH of greater than 7 and a temperature between **5°** and **50°** C, between a cathode and an opposed anode, which anode comprises an electrically conductive supporting substrate bearing on at least a portion of the surface thereof a coating consisting essentially of from **30** to **90** percent stannic oxide, from **1.0** to **10** percent antimony oxide, calculated as  $\text{Sb}_2\text{O}_3$ , from **1.0** to **50** percent of at least one platinum group metal oxide and from **0.5** to **30** percent of a valve metal oxide selected from the group consisting of titanium and tantalum oxides, with the proviso that the mole ratio of  $\text{SnO}_2:\text{Sb}_2\text{O}_3$  is between **95:5** and **85:15**.

**3.** A process as in claim 2 wherein the electrolyzing current is within the range of **0.5** to **1.0** ampere per square inch.

**4.** A process as in claim 2 wherein the alkali metal chloride concentration is between **28** and **35** grams per liter.

\* \* \* \* \*